

## UNITED STATES PATENT OFFICE.

COLIN G. FINK, OF YONKERS, NEW YORK, ASSIGNOR TO GUGGENHEIM BROTHERS, OF NEW YORK, N. Y., A COPARTNERSHIP.

## ELECTROLYTIC REFINING OR DEPOSITING OF TIN.

No Drawing.

Application filed February 1, 1922. Serial No. 533,249.

*To all whom it may concern:*

Be it known that I, COLIN G. FINK, a citizen of the United States, residing at Yonkers, in the county of Westchester, State 5 of New York, have invented certain new and useful Improvements in Electrolytic Refining or Depositing of Tin; and I do hereby declare the following to be a full, clear, and exact description of the invention, 10 such as will enable others skilled in the art to which it appertains to make and use the same.

This invention relates to the electrodeposition of tin and more particularly to the 15 electrolytic refining of tin. The invention has as its general object the provision of certain improvements in the electrodeposition of tin, and particularly contemplates the provision of an improved method of refining 20 tin electrolytically in which use is made of an electrolyte from which the tin is deposited in a more satisfactory physical condition than by the methods heretofore generally practiced in this art.

25 Considerable difficulty has heretofore been encountered in the electrodeposition and in the electrolytic refining of tin on account of the tendency of the tin to deposit from the electrolyte in the form of long crystals 30 which build up into "trees" or projections and eventually short-circuit the electrodes. Various expedients, such as diaphragms, electrolytes of special composition, etc., have been suggested from time to time for over- 35 coming this difficulty, but, as far as I am aware, the problem has not heretofore been satisfactorily solved from a practical stand-point. Diaphragms are objectionable because they introduce an added complication 40 into the electrolytic cell, and their elimination is, of course, desirable. Such electrolytes as have heretofore been suggested for the electrodeposition of tin, while they do in certain instances overcome the formation 45 of "trees" on the cathode, possess, nevertheless, other disadvantages, such, for example, as commercially unstable or expensive electrolytes (oxalates, fluosilicates, etc.) as well as deposits of impractical physical form.

50 Tin is deposited from neutral or alkaline

electrolytes in a finely granular or spongy condition. Such a deposit is found in practice to be very difficult and expensive to handle. On the other hand, tin is deposited from ordinary acid electrolytes in the form 55 of large crystals which build up to form "trees" and eventually short-circuit the electrodes. Acid electrolytes containing halogen ions (for example, hydrochloric acid or a suitable chloride) have been used to a 60 considerable extent in the electrodeposition of tin. In general, I have found that such acid electrolytes containing halogen ions give rise to very long crystals of tin which build up into "trees" and short-circuit the 65 electrodes after a comparatively short time of operation. Certain organic addition agents when introduced into such a halogen-containing electrolyte will reduce the size 70 of the deposited tin crystals, but large quantities of addition agents are required to produce deposits which can be readily handled in practice without mechanical loss.

75 As the result of my investigations and researches, I have found that a satisfactory smooth coherent deposit of tin can be obtained under commercial operating conditions by electrolyzing an aqueous bath containing an appropriate tin compound and a preponderating concentration of sulfate ions 80 and a preponderating concentration of ions of a metal more electropositive than tin, such as sodium, magnesium, iron, titanium or aluminum. The electrolyte which I use in practicing the invention is an aqueous 85 solution containing, for the most part, sulfuric acid, tin sulfate and an alkali, alkaline earth, or other suitable sulfate. This electrolyte contains a preponderating concentration of sulfate ions (anions), that is to say, 90 there is present in the electrolyte an excess of sulfate ions as compared with other anions present so that the major part of the electric current in the direction of the anode is carried by the sulfate ions. Small 95 amounts of chlorine, fluorine or silico-fluorine ions are not prejudicial to the final result, and the electrolyte may therefore contain a small amount of anions other than sulfate ions, such, for example, as chlorine, 100

fluorine, etc. In addition, the electrolyte employed in practicing the present invention contains a preponderating concentration of ions of a metal more electropositive than tin, such for example, as sodium, magnesium, iron, aluminum, etc. Inasmuch as these metal ions are more electropositive than tin, the tin is electrically deposited on the cathode or cathodes in preference to the 10 more electropositive metal ions contained in the electrolyte. In general, I have found that satisfactory results are obtained when the electrolyte contains 2 to 15 ions of sodium or other metal more electropositive than tin for each ion of tin in the electrolyte (assuming for convenience in explanation and definition complete disassociation of the salts in solution).

In actual practice, an electrolyte of substantially the following composition has given excellent results:

233 grams Glauber's salt ( $\text{Na}_2\text{SO}_4 \cdot 10\text{H}_2\text{O}$ ) per liter.

150 grams sulfuric acid per liter.

35 grams tin per liter.

2 grams aloin per liter.

In general, the principal substances in the foregoing electrolyte may be varied in about the following proportions:

30 Glauber's salt ( $\text{Na}_2\text{SO}_4 \cdot 10\text{H}_2\text{O}$ ) 50-350 grams per liter.

Concentrated sulfuric acid 50-150 grams per liter.

Tin 12-40 grams per liter.

35 Aloin 1-3 grams per liter.

In each of the foregoing formulæ the tin present in the electrolyte is calculated as metallic tin, although it is probably present in the electrolyte as stannous sulfate ( $\text{SnSO}_4$ ).

40 It is very probable that the sodium sulfate and the stannous sulfate form a double salt structurally resembling the alums.

Sulfuric acid alone is not well adapted for use in tin-containing electrolytes, because with such an electrolyte a very crystalline deposit of tin is produced. Furthermore, sulfuric acid alone is inoperative in the case of tin anodes containing appreciable quantities of lead as impurity. Sodium sulfate, 50 on the other hand, when used alone in a tin-containing electrolyte tends to give a spongy deposit of tin. However, when sulfuric acid and sodium sulfate are used together in the tin-containing electrolyte, the aforementioned defects of each substance alone are so neutralized that a dense, hard, finely crystalline deposit of tin is obtained.

I prefer to use sodium sulfate or Glauber's salt in preparing the electrolyte for carrying out the present invention because of its availability and cheapness. However, the sodium sulfate may be replaced either wholly or in part by magnesium sulfate, iron sulfate, aluminum sulfate, or by any sulfate of a metal more electropositive than tin. Thus,

the electrolyte may contain sodium and magnesium sulfates, or sodium, magnesium, and iron sulfates, or sodium, iron and chromium sulfates, the combined amount of such metal sulfates being present in the electrolyte in about the molecular equivalent of the proportions hereinbefore mentioned with respect to Glauber's salt.

Aloin is a glucoside obtained from aloes and varies more or less in chemical composition and physical properties according to the source from which it is obtained. It is chiefly prepared from Curacao aloes.

Aloin, as an addition agent in tin electrolytes, assists in preventing the formation of needle-like crystals. Instead of aloin, similar glucosides or organic colloids, such for example, as saponin, digitalis, cascara sagrada, cresylic acid, henna, gelatin, glue, tannic acid, or the like, may, if desired, be used as the addition agent. However, of a large number of addition agents with which I have experimented, aloin is the most satisfactory, and I therefore prefer to employ this substance in some form or other (for example, in the form of an extract from Curacao aloes) in the practice of the present invention. Gelatin and cresylic acid-soap emulsion, as addition agents, have temporarily produced very satisfactory electrolytic deposits of tin, but the activity of these agents appears to be quickly destroyed. On the other hand, aloin, as an addition agent, remains active for a relatively long period of time. Moreover, aloin may be cheaply obtained from Curacao aloes, the hot water extract from Curacao aloes containing the desired essential constituents of aloin and to nearly the same extent.

Very satisfactory practical deposits of tin are obtained at room temperature from electrolytes of the general composition hereinbefore discussed. In general, temperatures around 20° centigrade have been found entirely satisfactory. Temperatures lower than 20° C. cause a further refinement in the crystalline grain of the deposited tin, but such further advantages are of little material value in commercial practice. Temperatures much above 20° C. cause coarsening of the crystalline grain and a tendency towards irregularity of the deposit. In general, satisfactory results are secured when the temperature of the electrolyte is between 15° to 25° C. (60-80° F.). On account of the low electric potential and consequent low heating effect of the current it is not difficult to maintain the electrolyte at 15° to 25° C.

In practicing the invention, impure tin is made the anode and the cathode may advantageously be made up of tin foil. No diaphragms are required in the electrolytic cell. The voltage required is low; a voltage drop of around 0.2 volts, or even less, being satisfac-

tory. The current density may advantageously be about 10 amperes per square foot. The method of electrodepositing tin in accordance with the present invention is one of marked economy in current consumption, and in addition gives a satisfactory tin deposit. Moreover, the method of the invention can be continuously practiced over long periods of time without objectionably short-circuiting the electrodes.

The main advantages of electrodepositing tin in accordance with the method of the invention may be briefly summarized as follows:

- 15 1. Relatively low cost of the electrolyte.
2. Firm, dense, finely crystalline deposit of tin which makes it possible to turn out relatively thick cathodes without "treeing" and short-circuiting of electrodes.
- 20 3. No artificial heating of electrolyte is required, ordinary room temperatures being satisfactory.
4. No diaphragms are required.
5. The impurities in the anode tin, such as 25 antimony and bismuth, form sludges which are easily removed.

The method of the present invention is well adapted for use in the electrolytic refining of tin produced by the reduction of 30 oxidized tin ores with a gaseous reduction agent, such as hydrogen, carbon monoxide, or the like, at relatively low temperatures, as described in my application for Letters Patent of the United States Serial No. 452, 35 951 filed March 17, 1921. Where the reduced tin is recovered in metallic state, for example, as cast impure tin, such cast tin can be used as the anode in the electrolytic refining process. If the reduced tin is of a 40 porous or a granular character, it may be compressed and then used as the anode.

The impurities contained in anodes produced as described in the preceding paragraph from Bolivian tin ores will vary somewhat, but usually lead, bismuth and antimony are present in appreciable amount, and small amounts of arsenic, iron and copper may also be present. The impurities, particularly the bismuth and antimony, tend 45 to remain behind on the anodes or to form a sludge which settles to the bottom of the electrolytic apparatus.

As previously stated, small amounts of 55 chlorides, fluorides or the like, present in the electrolyte of the invention, are not prejudicial to the final result. The amount of such substances present in the electrolyte will, however, always be relatively small in comparison with the amount of sulfate ions 60 present in the electrolyte because, in accordance with the main principle of the present invention, the electrolyte contains a preponderating concentration of sulfate ions and may or may not, as the case may be, 65 contain relatively small amounts of other

anions, such as chlorides, bromides, fluorides, and the like. In addition, the electrolyte of the invention contains a preponderating concentration of ions of a metal or metals more electropositive than tin.

Where the crude anode tin contains around 2% or more of lead, I find it of advantage to employ reduced amounts of sulfuric acid in the electrolyte. Thus, the acid may to this end be reduced to 50 grams per liter. Reduction (below about 100 grams per liter) in the acid causes the cell voltage to rise, and consequently it is a very important consideration that as high acidity as possible be used in order to keep the power costs down. A further objectionable feature of low acidity is the tendency for spongy deposits to form on the cathode. Likewise, it has been found advantageous with high lead anodes to reduce the concentration of 80 the Glauber's salt to one-half or one-fourth the 233 grams per liter hereinbefore recommended. The Glauber's salt may be replaced by other salts such as ferrous sulfate, without greatly impairing the quality of 85 the cathode deposit, yet greatly improving the anode corrosion. I have found that from about 50 to about 100 grams per liter of Glauber's salt gives the best results as regards anode corrosion and cathode deposition.

I have also found that the addition to the electrolyte (hereinbefore described) of certain metal sulfates (herein called "additional metal sulfates") such as sulfates of iron, titanium, cobalt, nickel, manganese and chromium, produce a beneficial result. These metal sulfates appear to play a two-fold part in the tin-refining cell. In the first place, their presence has the effect of loosening the slimes coating from the anode, thus rendering corrosion of the anode more easy. In the second place, the presence of these metal sulfates effects a marked improvement in the density, hardness and blend of the tin crystals deposited on the cathode. This has been found especially true of nickel, iron and chromium. I have secured satisfactory results by the addition to the electrolyte of 10 to 20 grams of iron (in the form of ferrous sulfate) or 1 to 3 grams of chromium (in the form of chromous sulfate) per liter, or both iron and chromous sulfates. Such metallic sulfates (for example, ferrous sulfate, nickelous sulfate, chromous sulfate, etc.) may, however, be present in the electrolyte in an amount up to 30 grams (calculated as metal) per liter for imparting to the electrolyte the advantageous properties just mentioned. Acetic acid has also been found to impart to the tin electrolyte advantages similar to those resulting from the addition of the aforementioned metal sulfates.

The addition of iron and chromous sul-

ates is particularly beneficial in case the anodes contain lead and bismuth as high as 2% or 3%. If the anode tin is very impure and carries much over 3% lead, I prefer to give the molten tin a preliminary treatment before casting into anodes. Blowing the molten anode tin with oxygen or air will reduce the lead content very easily. Addition of sulfur to the molten bath has a similar effect. However, I find that the most reliable procedure, giving uniformly good results during refining later on, is to add to the molten anode tin bath from 0.1% to 1.5% aluminum metal. The ratio of lead to tin should be approximately ten to one. I have found that lead tin anodes containing as much as ten per cent of lead and about two per cent of bismuth would give rise to no polarization voltages during the course of refining the tin; the anodes would dissolve completely without any irregularities in the voltage performance. The presence of the aluminum metal in the tin anode causes the slimes to be comparatively loose, and any lead sulfate formed during electrolysis does not cling to the face of the anode as is likely to be the case in the absence of aluminum. Other metals besides aluminum have been tried but the results are not anywhere as good.

I claim:

1. The improvement in the electrodeposition of tin, which comprises depositing the tin from an electrolyte containing a preponderating concentration of sulfate ions with respect to other anions therein and a concentration of ions of a metal more electropositive than tin preponderating with respect to other cations therein.
2. The improvement in the electrodeposition of tin, which comprises depositing the tin from an electrolyte containing a preponderating concentration of sulfate ions with respect to other anions therein, and a concentration of sodium ions exceeding the concentration of tin ions therein.
3. The improvement in the electrodeposition of tin, which comprises depositing the tin from an electrolyte containing a preponderating concentration of sulfate ions with respect to other anions therein and a concentration of magnesium ions exceeding the concentration of tin ions therein.
4. The improvement in the electrodeposition of tin which comprises depositing the tin from an electrolyte containing a preponderating concentration of sulfate ions with respect to other anions therein and containing a concentration of sodium- and magnesium ions preponderating with respect to other cations therein.
5. The improvement in the electrodeposition of tin, which comprises depositing the tin from an electrolyte containing a preponderating concentration of sulfate ions with

respect to other anions therein and a preponderating concentration of sodium ions with respect to other cations therein.

6. The improvement in the electrodeposition of tin, which comprises depositing the tin from an electrolyte containing sulfuric acid and sodium sulphate in preponderating amounts as compared with the amounts of other substances contained in the electrolyte.

7. The improvement in the electrodeposition of tin, which comprises depositing the tin from an electrolyte containing sulfuric acid and the sulfate of a metal or metals more electropositive than tin in preponderating amounts as compared with the amounts of other substances contained in the electrolyte.

8. The improvement in the electrodeposition of tin, which comprises depositing the tin from an electrolyte containing in each liter thereof from 50-150 grams of sulfuric acid and from 50-350 grams of Glauber's salt.

9. The improvement in the electrodeposition of tin, which comprises depositing the tin from an electrolyte containing a preponderating concentration of sulfate ions with respect to other anions therein, and a concentration of ions of a metal more electropositive than tin preponderating with respect to other cations therein and also containing aloin as an addition agent.

10. The improvement in the electrodeposition of tin, which comprises depositing the tin from an electrolyte containing sulfuric acid and the sulfate of a metal or metals more electropositive than tin in substantially the following proportions: Sulfuric acid 50 to 150 grams, metal sulfate or sulfates, the molecular equivalent of 50 to 350 grams of Glauber's salt per liter.

11. The improvement in the electrodeposition of tin, which comprises depositing the tin from an electrolyte containing from 50 to 150 grams per liter of sulfuric acid and from 50 to 350 grams per liter of the sulfate of a metal or metals more electropositive than tin and up to 30 grams per liter (calculated as metal) of one or more of the hereinbefore mentioned additional metal sulfates.

12. The method of refining tin electrolytically, which comprises depositing the tin from an electrolyte containing sulfuric acid and sodium sulfate.

13. The method of refining tin electrolytically, which comprises depositing the tin from an electrolyte containing sulfuric acid and magnesium sulfate.

14. The method of refining tin electrolytically, which comprises depositing the tin from an electrolyte containing stannous sulfate, sulfuric acid, sodium sulfate and an addition agent.

15. The method of refining tin electro-

lytically, which comprises passing a current of low voltage from an impure tin anode to a cathode, the electrolyte containing stannous sulfate, sulfuric acid, sodium sulfate, and aloin.

16. The method of refining tin electrolytically which comprises subjecting reduced tin ore to compression, placing the tin thus

compressed in an electrolytic bath, and passing a current through said compressed tin, 10 the electrolyte and a cathode.

17. An anode for use in the electrolytic refining of tin, comprising compressed, relatively impure, reduced tin ore.

In testimony whereof I affix my signature.  
COLIN G. FINK.